

## UNITED STATES PATENT OFFICE

2,168,574

## METHOD OF SEPARATING WAX-CONTAINING MATERIALS

Dwight B. Mapes and Eddie M. Dons, Tulsa, Okla., assignors to Mid-Continent Petroleum Corporation, Tulsa, Okla., a corporation of Delaware

No Drawing. Application May 10, 1937,  
Serial No. 141,860

## 4 Claims. (Cl. 196—18)

This invention relates to methods of separating wax-containing materials, the present application being a continuation in part of an application filed by us on May 20, 1936, Serial No. 80,672.

5 An object of the invention is to produce a highly efficient method of separating various wax-containing materials, including lubricating oil stocks, as well as petrolatum, slack wax and other mixtures containing high and low melting

10 point waxes.

A further object is to produce an economical and entirely feasible method of this kind, without incurring any of the serious undesirable factors involving time, trouble or expense to be expected at one or more stages of an otherwise desirable dewaxing process. Actual tests of the invention have shown that it overcomes all of these problems.

More specifically stated, an object is to accomplish the above mentioned results in a simple process, while employing a new combination of inexpensive solvents that can be safely used without incurring any serious danger of fire, explosion, or the like, and which cooperate with each other to provide a high filter rate, large yields of the wax or oil, and excellent quality in the resultant products.

With the foregoing and other objects in view, the invention comprises the novel methods hereinafter described to set forth specific examples of the invention. However, it is to be understood that this invention comprehends changes, variations and modifications within the scope of the claims hereunto appended.

35 Prior to our inventions in this art, it has been customary to employ combinations of radically different solvents, the general rule being to select one solvent having a high solvent power for one of the constituents to be separated, and another solvent having a low solvent power for that constituent, but a high solvent power for another constituent. For example, in accordance with the theory generally adhered to in the art, a solvent having a high solvent power for wax may be combined with a substantially different solvent deliberately selected because it has a low solvent power for wax.

Instead of employing such radically different solvents, we prefer to use a combination of solvents of the same general class, and in practice we have found that the particular solvents herein set forth actually produce the entire series of desirable results, despite the similarity in the general nature of the cooperating solvents.

55 Propyl acetate alone may be used as a dewax-

ing solvent to produce low cold test lubricating oils, and also to separate the various waxy materials, or to remove oil from such waxy materials. We have used this single solvent in dewaxing lubricating oil stocks, and for deoiling petrolatum. Propyl acetate has outstanding merit as a simple solvent for work of this kind. Owing to its relatively low cost, we prefer to use isopropyl acetate, instead of the normal propyl acetate.

However, in the preferred form of the invention, we employ a blend of propyl acetate and another fatty acid ester of an aliphatic alcohol, and thereby accomplish important results not obtainable from the propyl acetate alone.

When the propyl acetate contains water, and this may be expected of propyl acetate recovered in the usual manner by distillation in the presence of steam, we have found that certain specific objections appear in the use of this otherwise desirable solvent. In using such propyl acetate as a solvent for deoiling petrolatum, we found that soft waxes, or gel-like materials of an adhesive nature are thrown out of solution, resulting in a very undesirable sticky wax cake which adheres to the filter, and that the objectionable oil, etc., can not be washed from this sticky wax. Similar effects were observed in using propyl acetate to dewax lubricating oil stocks containing amorphous wax.

However, by adding amyl acetate to the propyl acetate, we overcome this problem, and produce a very high yield of commercially desirable wax in the form of a porous hard cake that can be very easily washed on the filter.

Amyl acetate has been previously employed as a dewaxing solvent, but amyl acetate when used alone would result in low filter rates and produce an objectionable bulky and oily wax cake. Amyl acetate alone would be quite unsatisfactory, and not desirable for a commercial process of this kind. Nevertheless, the mixture of propyl acetate and amyl acetate precipitates the wax in a more sharply defined crystalline form, which permits rapid filtration, and the wax cake is more compact and more free of oil. This wax cake is very readily washed to produce a dry cake having a very low oil content.

More specifically stated, as an example of the new process used in deoiling petrolatum, we prepared a solvent composed of 70% isopropyl acetate and 30% technical grade amyl acetate, using five parts of this solvent to one part petrolatum. The solution was heated to about 135° F., then cooled to 76° F. and filtered. The wax cake on the filter was washed with a quantity of solvent

equal to .6 to .7 of the volume of the original petrolatum. This resulted in a large yield of the most valuable wax having a high melting point of 160° F., which was about 40% of the original stock.

This combination of propyl acetate and amyl acetate is especially desirable for deoiling petrolatum, as the petrolatum contains the soft waxes, or gel-like sticky material, most undesirable in the finished product. We have found that the new combination of solvents is quite selective in holding these adhesive soft waxes in solution, and in producing a high yield of the hard wax. The wax thus precipitated is quite free of said sticky material, and forms a very compact wax cake on the filter. This cake can be readily washed, and easily discharged from the filter, the resultant product being an excellent clean hard wax.

As another specific example of the invention, we will now refer to the dewaxing of a lubricating oil stock to produce an oil having a low pour point. The solvent was composed of 90% isopropyl acetate and 10% amyl acetate. The oil stock was a blend of 40% petroleum residue and 60% distillate having a viscosity of 95 at 210° F. The oil stock was dissolved in this solvent and the solution was chilled and then filtered. The solvents were distilled from the oil in the presence of steam, and used in subsequent operations. The resultant oil was a finished bright stock having a viscosity of 125 at 210° F. The cloud point of this oil was -20° F., which shows that all of the wax was removed.

In the foregoing example, the solution was filtered at 10° F., and the dewaxed oil had a pour point of -5° F. Actual tests of the invention herein disclosed have positively shown that the new method overcomes all of various serious defects or objections likely to arise unexpectedly in processes of this kind, and that it provides an economical and entirely feasible method of accomplishing the several results desired in this art.

The outstanding results derived from the cooperative action of propyl acetate and amyl acetate are quite apparent in deoiling or dewaxing petroleum stocks containing amorphous wax, and particularly in obtaining the valuable high melting point wax from petrolatum, which involves a number of specific problems not present in the separation of paraffin waxes. Nevertheless, we have found that the combination of these two solvents is also desirable in separating various stocks containing paraffin waxes, and said solvents can be advantageously employed in purifying slack wax, in lieu of the usual sweating

operations. For example, in separating slack wax, using isopropyl acetate and amyl acetate as a combined solvent, we obtained a yield of wax having a melting point of 122° F. amounting to 40% of the original stock, whereas the usual sweating resulted in a 28% yield of wax having the same melting point. By using said combination of solvents we have economically separated the higher melting point waxes from slack wax, which are not obtainable by sweating.

The proportions of the solvents may be varied as desired, depending upon the stock to be treated and the results to be obtained. The propyl acetate is preferably from about 40% to about 90% of the solvent blend, and the dewaxing may be carried out at high temperatures above 50° F., for example, about 75° F. to recover high melting point wax from petrolatum; or in making low pour point oils, the dewaxing may be performed at relatively low temperatures. However, the invention is not limited to the specific temperature conditions, nor to the range of proportions specifically mentioned in referring to the solvents.

We claim:

1. The method of separating wax-containing materials derived from petroleum which comprises dissolving said materials in a solvent comprising isopropyl acetate and amyl acetate, cooling the solution to precipitate wax therein, and separating wax from the cooled solution.

2. In the art of separating amorphous wax from petroleum stocks containing said wax and oil, the method of using isopropyl acetate which comprises dissolving said petroleum stocks in a solvent including said isopropyl acetate and amyl acetate, cooling the solution to precipitate wax therein, and separating precipitated wax from the cooled solution.

3. The method of separating high melting point wax from petroleum stocks containing amorphous wax and oil which comprises dissolving the waxy material in a solvent including isopropyl acetate and amyl acetate, cooling the solution to precipitate high melting point wax therein, and separating precipitated wax from the cooled solution.

4. In the art of deoiling petrolatum, the method of using isopropyl acetate which comprises dissolving the petrolatum in a solvent including said isopropyl acetate and amyl acetate, cooling the solution to precipitate high melting point wax therein, and separating precipitated wax from the cooled solution.

DWIGHT B. MAPES. 55  
EDDIE M. DONS.